# EUROPEAN PATENT APPLICATION

(11) **EP 0 949 085 A2**
(43) Date of publication of application: **13.10.1999**
(21) Application number: 99302731.7
(22) Date of filing: 07.04.1999
(51) Int. Cl.: B41M 5/035, B41M 5/38

(54) **Thermal transfer printing on plastics materials**

(30) Priority: 07.04.1998 GB 9807436
(71) Applicant: BOWTHORPE PLC, Crawley, West Sussex RH10 2RZ (GB)
(72) Inventor: Haggarty, John Nicholas, Milehouse, Plymouth PL2 3AX (GB)
(74) Representative: Davies, Gregory Mark

(57) **Abstract**

A printed marking on a plastics substrate has a first, sub-surface portion of a first pigmentation material bound to, or penetrated into the substrate, and a second, surface portion of a second pigmentation material adhered to the surface of the substrate overlaying the sub-surface portion of the mark. The dual nature of the marking provides advantages in terms of durability, particularly for use in harsh environments , or situations where the mark is liable to be subject to chemical action, or abrasion in the normal course of events or in cases of unauthorised tampering.

## Description

The present invention relates to marking plastics substrates and in particular to marking plastics substrates using a thermal transfer printing process.

Printed markers comprising plastics substrates printed with indicia conveying data are known and widely used. For example printed plastics sheaths or flat strip tags are widely used for identifying electric cables. The known types of sheaths or strip tags are passed in unprinted "feedstock" form through conventional thermal transfer printing apparatus in order to be marked with the required predetermined indicia. In conventional thermal transfer printing, pressure and heat are applied to a printing ribbon registering against the plastics feedstock, such that a print composition carried by the ribbon is transferred to the feedstock. Conventionally, thermal transfer ribbons rely upon a wax or resin to transfer the dry ink onto the feedstock substrate.

This method of marking has inherent drawbacks; for example, the ink can be removed by means of heat, chemical action or abrasion. This can result in important printed markers becoming unreadable. Furthermore, over time, the action of ultra violet radiation on pigments in the ink can result in the mark fading.

Improvements have now been devised to marking plastics substrates.

According to a first aspect, the invention provides a thermal transfer printing process for marking a plastics substrate, the process comprising applying heat and pressure to a print carrier registering against the substrate resulting in transfer of a printing composition carried by the print carrier to the substrate, the printing composition comprising a first pigmentation material arranged to bind to or penetrate into the plastics substrate to form a substantially permanent mark below the surface of the substrate, and a second pigmentation material arranged to adhere to the surface of the substrate overlaying the substantially permanent mark.

The invention enables a single stage printing process to be used to print a marking of predetermined configuration onto a plastics substrate comprising a sub-surface marking and corresponding surface printed marking simultaneously. The dual nature of the marking provides advantages in terms of durability, particularly for use in harsh environments , or situations where the mark is liable to be subject to chemical action, or abrasion in the normal course of events or in cases of unauthorised tampering.

The invention is particularly suitable for use in providing plastics printed markers for identifying articles. According to a second aspect the invention therefore provides a plastics printed marker comprising a plastics substrate having a printed mark, the printed mark comprising:
a) a first, sub-surface portion of a first pigmentation material bound to, or penetrated into the substrate, and;
b) a second, surface portion of a second pigmentation material adhered to the surface of the substrate overlaying the sub-surface portion of the mark.

The printing composition carried by the print carrier comprises the first and second pigmentation materials and also, preferably, a plastics material facilitating binding with or penetration into the substrate. It is believed that a print carrier carrying such a printing composition is both novel and inventive per se, and thus provides a further aspect of the invention. This is particularly believed to be the case for such a print carrier for use in thermal transfer printing onto plastics substrates.

In one embodiment, the plastics material comprising the printing composition may be the same as the plastics material comprising the substrate.

In an alternative embodiment, the plastics material comprising the print composition may be different from the plastics material comprising the substrate. In this instance, the plastics material transferred from the print carrier and bound with, or penetrated into, the substrate will be identifiable in the resulting printed marker, at least upon microscopic inspection.

It is preferred that the plastics material carried by the print carrier comprises a thermoplastic material, such as PVC, a polyolefin or the like, more preferably, a homopolymer material.

The printed marker according to the invention preferably comprises a plastics strip or length of plastics tubing (which tubing may be heat shrinkable or non-heat shrinkable). Where the printed marker is in the form of plastics tubing, it is preferred that the feedstock is in the form of flattened tubing. This facilitates ease of printing.

It is preferred that the print carrier comprises a plastics film (desirably comprising polyester) preferably of a thickness substantially in the range 4-15 microns, more preferably approximately 6 microns. The print carrier is capable of separating from the print composition it carries during the thermal transfer printing process. Desirably the print carrier is wound from a reel store.

The print composition (or ink) carried by the print carrier is preferably touch dry. The first and second pigmentation materials are preferably relatively dark in colour and may for example be blue or black. The pigmentation materials may for example comprise dyes of suitable composition to ensure that one penetrates the substrate and the other adheres to the surface of the substrate during the printing process.

One or other (or both) of the first and second pigmentation materials may comprise a mixture or composition of a plurality of dyes.

It is preferred that the printing composition comprises the pigmentation materials and the plastics material bound in a matrix material. The printing composition is preferably applied to the print carrier as a layer. The matrix material may, for example, comprise a relatively soft, high molecular weight material such as a wax or wax-like material.

The thermal transfer printer may be arranged to print any predetermined indicia mark upon the substrate.

The invention will now be further described in a specific embodiment by way of example only and with reference to the accompanying drawings in which:
Figure 1 is a plan view of a first embodiment of marked substrate according to the invention;
Figure 2 is a schematic sectional view of a prior art marked substrate;
Figure 3 is a schematic view of thermal transfer printing apparatus for operating the process of the invention; and
Figure 4 is a schematic sectional view of a substrate marked in accordance with the invention.

Referring to the drawings, Figure 1 shows "feedstock" in the form of a length of flattened heat-shrinkable plastics tubing 1 (or sheathing) ; following printing of a respective portion of the tubing 1 a marked indicium 2 is identifiable on the surface.

Referring to Figure 2, when applying conventional thermal transfer printing techniques, a layer of printed ink 3 adheres to the surface of tubing 1. It is possible intentionally, or accidentally, to remove the printed ink layer 3 from the underlying plastics tubing substrate 4 by abrasion, chemical action or degradation due to exposure to ultra-violet radiation.

The apparatus for printing of the tubing substrate 1 is shown in Figure 3 and generally designated 4. The apparatus comprises a drive roller 35 which draws feedstock tubing 1 from a reel store (not shown) to extend past a thermal printing head 36 of the apparatus. Simultaneously, a printer ribbon 38 is fed from a store of unused ribbon 39 extending past printing head 36, subsequently being wound of reel 40. In use, the printing head 36 is urged to press against flattened feedstock tube 1 sandwiching printer ribbon 38 therebetween, such that printer ribbon 38 is held in register with the feedstock tubing 1. In this way, the relevant indicia are marked on the tubing 1 as the print composition carried by the printer ribbon 38 is transferred to the surface of the flattened tubing 1.

Printer ribbon 38 comprises a polyester backing film between 4-15 microns in thickness (preferably approximately 6 microns in thickness), and which is arranged to release the printing composition under the applied pressure and heat of the thermal printer head 36. The print composition carried by the printer ribbon 38 is dry to the touch and comprises first and second selected pigmentation materials (such as respective dyes) and a thermoplastic material compatible with the material of the tubing 1 carried in a suitable matrix material, such as wax.

One of the pigmentation materials, and also the thermoplastic material, are selected to bind with the plastics material of the tubing substrate, or penetrate into the plastics material of the tubing substrate (for example by diffusion), upon application of the thermal transfer printing head. In this way, as shown most clearly in figure 4, a substantially indelible mark 7 in the required configuration of the indicia is formed at, or more preferably below, the surface of the substrate material (wall of tubing 1) . The other of the pigmentation materials is selected-to be printable on the surface of the plastics tubing 1 substrate, and not to penetrate significantly below the substrate surface. This provides a surface printed mark 3 overlaying the subsurface mark 7.

A suitable printing composition and matrix for performance of the invention has been found to be as follows:
i) 50-70% by weight, first and second pigmentation materials. The first pigmentation material comprises a first dye (a solvent violet) based on N - tetra, N - penta, N - Lisea para-rosaniline hydrochlorides and a second dye (a solvent black) being an azo dye of formula C₂₉ H₂₄ N₆ chemical name 1 H - pyrimidine, 2,3 - dihydro - 2,2 - dimethyl - 6 [(4 - (phenylazo) - 1 - naphthyl) azo]. The second pigmentation material comprises an amorphous black inert solid such as furnace black.
ii) 8-12% by weight low molecular weight homopolymer PVC.
iii) 15-20% by weight, releasing agent comprising a wax (stearic acid).

The constituents of the printing composition are milled together; the combined material is then layered onto the polyester film.

In use, the first pigmentation material binds with the PVC nomo polymer material and penetrates the material of the plastics tube 1 to provide the subsurface mark 7. The second pigmentation material provides the surface printed mark 3 overlaying the subsurface mark 7.

The invention provides a single stage printing process for printing a high quality and substantially indelible mark upon plastics substrates. The printed mark does not require fixing (which is often necessary with prior art techniques) and has good resistance to fading under ultra-violet radiation. The printer ribbon can be used with conventional thermal transfer printing apparatus.

## Claims

1. A thermal transfer printing process for marking a plastics substrate, the process comprising applying heat and pressure to a print carrier registering against the substrate resulting in transfer of a printing composition carried by the print carrier to the substrate, the printing composition comprising a first pigmentation material arranged to bind to or penetrate into the plastics substrate to form a substantially permanent mark below the surface of the substrate, and a second pigmentation material arranged to adhere to the surface of the substrate overlaying the substantially permanent mark.

2. A print carrier carrying a releasable printing composition, which print composition comprises a first pigmentation material capable of binding to or penetrating into a plastics substrate, and a second pigmentation material capable of adhering to the surface of the plastics substrate.

3. A printing process or a print carrier according to claim 1 or claim 2, wherein the printing composition carried by the print carrier comprises the first and second pigmentation materials and also a plastics material facilitating binding with or penetration into the substrate;
preferably wherein the plastics material comprising the printing composition comprises:
plastics material substantially identical to the plastics material comprising the substrate; or
plastics material substantially different from the plastics material comprising the substrate.

4. A process or a print carrier according to any preceding claim, wherein the plastics material carried by the print carrier comprises a thermoplastic material (preferably a homopolymer material).

5. A process or a print carrier according to any preceding claim, wherein:
i) the print carrier comprises a plastics film, preferably wherein the print carrier comprises a polyester film; and/or
ii) wherein the print carrier is of a thickness substantially in the range 4-15 microns, preferably of approximately 6 microns.

6. A process or a print carrier according to any preceding claim, wherein the print carrier is capable of separating from the print composition during the thermal transfer printing process; and/or
wherein the print carrier is wound from a reel store; and/or
wherein the print composition (or ink) carried by the print carrier is touch dry; and/or
wherein the first and second pigmentation materials are relatively dark in colour; and/or
wherein one or other (or both) of the first and second pigmentation materials may comprise a mixture or composition of a plurality of dyes; and/or
wherein the printing composition comprises the pigmentation materials and the plastics material bound in a matrix material, the matrix material preferably comprising a relatively soft, high molecular weight material such as a wax or wax-like material.

7. A process or a print carrier according to any preceding claim, wherein:
i) the pigmentation material comprises dyes of suitable composition to ensure that one penetrates the substrate and the other adheres to the surface of the substrate during the printing process; and/or,
ii) the substrate comprises a plastics strip or length of plastics tubing (the feedstock preferably being in the form of flattened tubing).

8. A process or a print carrier according to any preceding claim, wherein:
the print carrier carries:
i) 50-70% by weight, first and second pigmentation materials;
ii) 8-12% by weight plastics material (preferably comprising a low molecular weight homopolymer PVC) susceptible to binding with or penetrating into the substrate; and,
iii) 15-20% by weight, releasing agent/matrix material (preferably comprising a wax material such as stearic acid) ; and/or
the second pigmentation material comprises an amorphous black inert solid such as furnace black; and/or,
the printing composition is applied to the print carrier as a layer.

9. A process according to any preceding process claim, wherein the thermal transfer printer is arranged to print a predetermined indicia mark upon the substrate.

10. A plastics printed marker comprising a plastics substrate having a printed mark, the printed mark comprising:
a) a first, sub-surface portion of a first pigmentation material bound to, or penetrated into the substrate, and;
b) a second, surface portion of a second pigmentation material adhered to the surface of the substrate overlaying the sub-surface portion of the mark.

11. A plastics printed marker according to claim 10,
wherein the substrate comprises a plastics strip; and/or
wherein the substrate comprises a length of plastics tubing,
preferably wherein the first and second pigmentation materials are relatively dark in colour.
